

## UNITED STATES PATENT OFFICE

1,987,095

## SPINNING SOLUTIONS FOR THE MANUFACTURE OF SOFT-LUSTER RAYON

Rudolph S. Bley, Elizabethton, Tenn., assignor to North American Rayon Corporation, New York, N. Y., a corporation of Delaware

No Drawing. Application August 3, 1934,  
Serial No. 738,377

6 Claims. (Cl. 106—40)

- The present invention relates to a process of preparing cellulosic spinning solutions from which soft-luster filaments, yarns, ribbons, films, etc., may be formed.
- 5 The primary object of my invention has to do with the incorporation of an organic titanium compound into cellulosic spinning solutions which, upon extrusion or molding, yield soft-luster cellulosic products.
- 10 Another object of my invention is the incorporation of an organic titanium compound composition into viscose and cuprammonium spinning solutions, said composition consisting of  $(C_2H_5O)_2TiO.PH_3O_4$

15 dissolved and/or dispersed in an organic liquid inert to said spinning solution.

Other objects of my invention will become apparent to those skilled in the art after a study of the following specification.

20 In the early days of rayon manufacture, the demand was entirely for yarns having the highest possible degree of luster. Later, when it was found that highly lustrous rayon too clearly indicated its origin—an artificial fiber—a demand arose for 25 artificial silk which more closely approximated to natural silk. The earliest attempt to meet the demand of dull-luster viscose yarn, for example, was a method of retaining sulphur particles in the fibers by discontinuing the normal desulphurizing 30 step during its manufacture. Although this yarn showed decreased luster, due to scattering of light by the sulphur particles, it was impermanent and exhibited an unattractive "bloom". This method has been improved by dispersing, instead of sulphur, fine inorganic or organic particles in cellulosic spinning solutions, such as pigments, hydrocarbons and the like.

I am well aware that it has, heretofore, been proposed to incorporate inorganic and organic 40 titanium compounds into cellulosic spinning solutions to produce soft-luster yarns (vide U. S. Patents 1,692,372 and 1,791,199 to Gardner, U. S. Patent 1,875,894 to Singmaster, U. S. Patent 1,969,689 to Byron, British Patent 343,949 to 45 Dreyfus, etc.)

With exception of a special titanium oxalate, disclosed in the aforementioned U. S. Patent 1,969,689, to Thomas H. Byron of August 7, 1934, all of the titanium compounds, heretofore used in 50 the art, are somewhat alkali- and acid-soluble. For this reason considerable amounts of these titanium compounds are wasted during the manufacture of soft-luster rayon.

In accordance with my present invention, not 55 a titanium oxalate but a titanium compound hav-

ing the formula  $(C_2H_5O)_2TiO.PH_3O_4$  is used in combination with viscose and cuprammonium cellulose solutions to form after extrusion soft-luster, cellulosic products.

This titanium compound may be produced by reacting  $TiPCl_3$  or  $TiPCl_7O$  upon aliphatic alcohols to form intermediate compounds having the structures

$(CH_3O)_3TiCl.PH_3O_4$  and  $(C_2H_5O)_2TiCl.PH_3O_4$ , respectively. After hydrolyzing these gum-like 10 intermediates, an organic titanium compound is obtained, having the formula

$(C_2H_5O)_2TiO.PH_3O_4$ ,

which is soluble in alcohol, insoluble in water and 15 ether, insoluble in viscose and cuprammonium cellulose solutions as well as in the acid setting baths used in connection with such spinning solutions.

The compound, before being dispersed in the 20 cellulosic solutions, is finely ground in pebble or colloid mills. Instead of dispersing the titanium compound per se in the spinning solutions, it may first be dissolved or dispersed in an inert, organic liquid to accelerate its uniform distribution therein. Thus, the titanium compound may be dissolved in alcohols and, subsequently, the alcoholic 25 solution added to the spinning solution. Due to the fact that  $(C_2H_5O)_2TiO.PH_3O_4$  is insoluble in the spinning solutions, set forth above, it is precipitated therein in the form of extremely fine 30 particles which may be uniformly distributed in the cellulosic solutions by stirring, etc. It is also possible to first disperse the finely ground titanium compound particles in an organic liquid, such as 35 hydrocarbons, mineral, vegetable and animal oils, fats, etc., and then to emulsify this mixture with the spinning solutions. In this manner the final luster of the cellulosic products may be modified, 40 since the aforementioned liquids are delustering agents per se. It is to be noted, however, that only such organic liquids are suitable which are inert with respect to the spinning solutions and which do not deleteriously affect the final products. The amounts of titanium compound added to a 45 spinning solution may be varied practically at will, although I have found that additions of about 1 to 12% of  $(C_2H_5O)_2TiO.PH_3O_4$  are sufficient to produce soft-luster products.

## Example 1

From 1 to 12% of  $(C_2H_5O)_2TiO.PH_3O_4$ , calculated on the cellulose content, are added to a conventional viscose spinning solution in the form of 55 a fine dispersion. The titanium compound may be

first ground to microscopic fineness and then dispersed in the viscose solution, or it may be dissolved in an organic solvent prior to incorporation into said solution. Instead of dissolving the titanium compound, it may be ground and dispersed in an inert, organic liquid to form an organosol. This organosol is then emulsified with the viscose solution under continuous stirring. The loaded spinning solution is subsequently extruded into

10 conventional spinning baths.

*Example 2*

From 1 to 12% of  $(C_2H_5O)_2TiO.PH_3O_4$  are added to a conventional cuprammonium cellulose solution, the percentages of titanium compound being based upon its cellulose content. The titanium compound is incorporated into the cuprammonium cellulose solution in accordance with the methods set forth in Example 1.

20 It is to be emphasized that the amounts of titanium compound, set forth above, may be decreased or increased to vary the luster of the finished, cellulosic products, although excessive additions tend to weaken the tensile strength of the rayon and to clog the fine holes of the spinning nozzles.

Modifications may be made in details of the method and the product without departing from the spirit and scope of my invention as defined

30 by the appended claims.

I claim:

1. A spinning solution for the manufacture of soft-luster products comprising a solution of the

group consisting of viscose and cuprammonium cellulose and an organic titanium compound having the formula  $(C_2H_5O)_2TiO.PH_3O_4$ .

2. A spinning solution for the manufacture of soft-luster products comprising a solution of the group consisting of viscose and cuprammonium cellulose, an organic liquid inert to said solution, and an organic titanium compound having the formula  $(C_2H_5O)_2TiO.PH_3O_4$ .

3. A spinning solution for the manufacture of soft-luster products comprising a solution of the group consisting of viscose and cuprammonium cellulose and from 1 to 12 per cent of an organic titanium compound having the formula

$(C_2H_5O)_2TiO.PH_3O_4$

15

said percentages of titanium compound being calculated on the cellulose content of the solution.

4. A spinning solution for the manufacture of soft-luster products comprising a solution of the group consisting of viscose and cuprammonium cellulose, an organic liquid inert to said solution and from 1 to 12 per cent of an organic titanium compound having the formula

$(C_2H_5O)_2TiO.PH_3O_4$

25

said percentages of titanium compound being calculated on the cellulose content of the solution.

5. A viscose filament containing finely divided  $(C_2H_5O)_2TiO.PH_3O_4$ .

6. A cuprammonium filament containing finely divided  $(C_2H_5O)_2TiO.PH_3O_4$ .

RUDOLPH S. BLEY.

30